

## UNITED STATES PATENT OFFICE.

FRED W. ALPERS, OF MUSKEGON, MICHIGAN.

## POLISHING COMPOUND.

No Drawing.

Application filed June 26, 1924. Serial No. 723,549.

This invention relates to certain new and useful improvements in polishing compounds especially adapted for use on metal surfaces for producing a highly finished surface on metal either before or after a lapping treatment or grinding of the metal face.

Recently the so-called "lapping process" has been introduced for treatment of many automobile parts. This process, however, leaves a somewhat feathery or minutely roughened metal surface, which has to be removed in some manner in order to give the highly finished or smooth surface required, for instance on automobile piston pins or the cylinder bores. Various materials or abrasives have been used to produce these highly polished or smooth surfaces, the principal ingredient of which has generally been powdered emery. We have found, however, that the use of a finely ground or pulverized cementitious material as ordinary cement (hydrated lime and a number of other high temperature cements may be employed) as a polishing material in itself alone is capable of producing a fairly good surface.

The great advantages from the use of cement or similar material as a polishing substance, however, is not secured until the same is mixed with another regularly employed polishing or grinding material; for instance pumice stone. Further to enhance the value of the process a certain percentage of fuller's earth is also incorporated into the polishing material, but the final optimum results are not secured by the process until finely ground emery, and more especially the so-called Turkish emery, is incorporated as one of the ingredients of the compound.

We have found that cement, used as a vehicle or carrier, and any one of the above named polishing materials gives good results and we do not wish to confine our invention or compound to the use of the above four ingredients. Any combination of one or more of them in conjunction with cement or with a cementitious material, as noted, may be advantageously employed.

A mixture which we have found to give optimum results consists of 16 ounces of cement,  $1\frac{1}{2}$  ounces of pumice stone,  $1\frac{1}{2}$  ounces of Turkish emery and  $\frac{1}{2}$  ounce of fuller's earth.

The polishing material may be used according to any of the known methods employed for polishing or finishing of metal surfaces and in conjunction with any machine so employed.

The use of oils with the compound is, of course, essential. A mixture consisting of 50% of a cutting oil and 50% of kerosene has been advantageously employed and mixed with the other ingredients to produce a body of the consistency of paste, although the quantity of oil may be varied at will. While the compound is, of course, intended for mixture with a cutting oil or the like, it is to be understood that the manufacture thereof may embody alone the mixing of the several ground or pulverized ingredients, and may be sold in such form for subsequent mixing with a cutting oil, or the mixing with the oil may be accomplished at the initial compounding of the ingredients. The basic principle of this compound preferably embodies the combination of ingredients as above outlined, and while a compound formed of the proportions previously stated is capable of producing optimum results, it is to be understood that such proportions may be changed to suit different characteristics of metal surfaces, as well as the substitution of equivalent materials.

What is claimed as new is:—

1. A polishing compound including a finely ground mixture of cement, pumice stone, fuller's earth and emery.

2. A polishing compound including a finely ground mixture of cement, pumice stone, fuller's earth, emery and cutting oil.

3. A polishing compound including a finely ground mixture of the following ingredients in the proportions stated, to wit: cement, 16 ounces; pumice stone,  $1\frac{1}{2}$  ounces; fuller's earth,  $\frac{1}{2}$  ounce, and emery  $1\frac{1}{2}$  ounces.

4. A polishing compound including a finely ground mixture of the following ingredients in the proportions stated, to wit: cement, 16 ounces; pumice stone,  $1\frac{1}{2}$  ounces; fuller's earth,  $\frac{1}{2}$  ounce; emery  $1\frac{1}{2}$  ounces; and an oil embodying a mixture of cutting oil and kerosene.

In testimony whereof I affix my signature.

FRED W. ALPERS.